# EUROPEAN PATENT APPLICATION

(11) **EP 1 746 046 A1**
(43) Date of publication of application: **24.01.2007**
(21) Application number: 06116120.4
(22) Date of filing: 27.06.2006
(51) Int. Cl.: B65D 85/76, B65D 75/30

(54) **Vacuum skin package for cheese**

(30) Priority: 19.07.2005 EP 05106604
(71) Applicant: Cryovac, Inc., Duncan, S.C. 29334 (US)
(72) Inventor: Fanfani, Andrea, 20149, Milan (IT); Bellini, Laura, 26013, Crema (IT)
(74) Representative: De Carli, Elda

(57) **Abstract**

The invention relates to a vacuum skin package suitable for the packaging of respiring cheeses, like gassing cheeses and moulded cheeses. Said package comprises a support member and a flexible skin-forming film draped over the cheese product wherein the support member has an oxygen transmission rate in the range of from 80 to 500 cm³ /m²-day-bar at 23°C and 0% RH and the flexible film has an oxygen transmission rate greater than 60 cm³ /m²-day-bar at 23°C and 0% RH.

## Description

### Technical Field

The present invention relates to a vacuum skin package for the packaging of cheese. In particular the present invention relates to a vacuum skin package for the packaging of respiring cheeses and to a method for vacuum skin packaging a cheese product.

### Disclosure of Invention

Vacuum skin packaging is a process well known in the art for using a thermoplastic packaging material to enclose a food product. The vacuum skin packaging process is in one sense a type of thermoforming process in which an article to be packaged serves as the mold for a forming web. An article may be placed on a support member, that can be flat or shaped, e. g. tray-shaped, bowl- shaped or cup-shaped, and the supported article is then passed to a chamber where a top flexible film is drawn upward against a heated dome and the softened top flexible film is then draped over the article. The movement of the film is controlled by vacuum and/or air pressure, and in a vacuum skin packaging arrangement, the interior of the container is vacuumized before final welding of the top flexible film to the support member. In a vacuum skin package the upper heated film thus forms a tight skin around the product and is sealed to the support. Vacuum skin packaging is described in many references, including FR 1,258, 357, FR 1,286, 018, AU 3,491, 504, US RE 30,009, US 3,574, 642, US 3,681, 092, US 3,713, 849, US 4,055, 672, and US 5,346, 735.

The term "vacuum skin packaging" (hereinafter "VSP") as used herein indicates that the product is packaged under vacuum and the space containing the product is evacuated from gases at the moment of packaging. The top flexible film is sometimes referred to as "skin-forming" film.

Several hundreds of different kinds of cheese are produced today with different packaging requirements. Some cheese products, particularly semi-hard cheeses, like Swiss cheese, emit a significant amount of carbon dioxide over time as a consequence of their curing process. The evolved carbon dioxide must be allowed to escape the package in order to maintain the properties of the cheese and the integrity of the package. If not allowed to escape the evolved carbon dioxide collects inside the package creating a so-called "ballooning effect", which is perceived by the average consumer as a defect in the packaging and an indication of possible spoilage. These cheese types are often referred to as "gassing" cheeses.

On the other hand, moulded cheeses, such as blue cheese, require a type of packaging that allows them to "breathe", that is to exchange oxygen with the outer atmosphere, in order to maintain the moulds alive and therefore the flavour of the product unchanged.

The gassing cheeses and the moulded ones are herein referred to as "respiring" cheeses due to their gas exchange requirements.

Due to their different breathing requiremens gassing cheeses and moulded ones are typically stored and sold in different types of packaging. Gassing cheeses are generally available to the consumer in hermetic packages, often under vacuum or under a modified atmosphere. On the other hand moulded cheeses are mostly sold in non-hermetic packages, such as waxed paper wrappings.

It would be desirable to provide a common packaging system for both gassing and moulded cheeses having enough flexibility to adapt to the different respiration requirements of these products and which would not require burdensome inventory arrangements on the side of the cheese producer.

It has now been found that vacuum skin packaging can offer a solution to this need. In particular it has been found that by carefully selecting the oxygen barrier properties of the skin-forming film and of the support member it is possible to obtain a vacuum skin package for respiring cheese (both gassing and moulded) which guarantees the shelf-life and the optimal preservation of the organoleptic properties of the product. Advantageously by properly selecting the oxygen barrier properties of the support memebr of the package it possible to meet the different respiration rerquirements of gassing and moulded cheeses by changing the skin-forming film. Thus only a limited number of inventoried packaging materials is required to meet most respiring cheese requirements.

Of the prior art available in the field of VSP packaging only DE 4001272C relates to a skin-forming film for the vacuum skin packaging of gas-evolving products such as cheese, comprising an ionomer base material and an outside coating comprising an anionic copolymer dispersion based on vinylidene chloride and methyl acrylate and an aqueous dispersion of a vinyl chloride based copolymer. Said skin-forming film is described as having a carbon dioxide transmission rate of about 800 cm³ /m²-day-bar and an oxygen transmission rate of less than about 200 cm³ /m²-day-bar. No mention is made about the composition or the properties of the support member.

US 5,846,582 discloses the vacuum skin packaging of shingled food slices, among which cheese slices. However, cheese products sold in slice form generally have reached a stage of their curing process wherein no or negligible gases are evolved and thus have no demanding "breathing" requirements.

Accordingly, a first object of the present invention is a vacuum skin package of a cheese product wherein the support member has an oxygen transmission rate of 80 to 500 cm³ /m²-day-bar at 23°C and 0% relative humidity and the flexible film draped over the cheese product has an oxygen transmission rate greater than 60 cm³ /m²-day-bar at 23°C and 0% relative humidity.

A second object of the present invention is a method of making a vacuum skin package of the first object comprising the steps of: providing a support member, loading a cheese product over the support member, and draping a flexible film over the cheese product and over the support member and wherein the support member has an oxygen transmission rate of 80 to 500 cm³ /m²-day-bar at 23°C and 0% relative humidity and the flexible film draped over the cheese product has an oxygen transmission rate greater than 60 cm³ /m²-day-bar at 23°C and 0% relative humidity.

In its first aspect the present invention relates to a vacuum skin package comprising:
a) a support member;
b) a cheese product loaded onto said support member; and
c) a flexible film draped over the cheese product and enclosing said cheese product on the support member, characterized in that the support member a) has an oxygen transmission rate of 80 to 500 cm³ /m²-day-bar at 23°C and 0% relative humidity and the flexible film c) has an oxygen transmission rate greater than 60 cm³ /m²-day-bar at 23°C and 0% relative humidity.

The oxygen transmission rate (hereinafter "OTR") is measured according to ASTM D-3985 using an OX-TRAN instrument by Mocon. Unless otherwise stated the OTR values throughout the text refer to measures made at 23°C and 0% relative humidity (hereinafter "RH").

The OTR value of the support member is independent of the OTR value of the flexible skin-forming film, i.e. the two OTR values do not have to be the same.

It is known that the oxygen barrier properties of certain materials, such as (ethylene-co-vinyl alcohol) copolymers (EVOH) and polyamides, vary greatly with humidity, their OTR values generally increasing with increasing humidity. The OTR values of the support member and of the flexible skin-forming film may also have a different dependence from humidity the one with respect to the other.

The possibility of combining a support member and a skin-forming film having different oxygen transmission properties represents one of the advantages of the package of the present invention with respect to other cheese packages such as shrink bags or pouches. In fact it allows a greater flexibility in modulating the gas permeation properties of the overall package. For instance, gassing cheeses, like Swiss cheese, are better preserved in an environment that allows a moderate passage of oxygen whereas moulded cheeses, like blue cheese, are better preserved in an environment with significant oxygen transmission properties. With the package of the present invention it will be possible to meet these different requirements by changing for instance only the flexible skin-forming film.

Some examples of suitable combinations of oxygen transmission properties for the support member and the flexible skin-forming film are reported below, the numbers being OTR values at 23°C and 0% RH expressed in cm³/m²-day-bar.

Support 80-250 / Skin-forming film 60-300; Support 80-250 / Skin-forming film 100-200; Support 80-250 / Skin-forming film 150-500; Support 80-250 / Skin-forming film 500-1000; Support 250-350 / Skin-forming film 60-300; Support 250-350 / Skin-forming film 100-200; Support 250-350 / Skin-forming film 150-500; Support 250-350 / Skin-forming film 500-1000.

OTR values of the skin-forming film can in some cases be as high as 10,000 cm³/m²-day-bar and even higher.

More specifically, shelf-lives in the order of 9 weeks, can be obtained for a moulded type cheese like Roquefort by combining a support member with an OTR in the range of 80 to 500 cm³/m²-day-bar, preferably in the range of 80 to 250 cm³/m²-day-bar, with a skin-forming flexible film with an OTR in the range of 500-1000 cm³/m²-day-bar, preferably in the range of 600 to 1000 cm³/m²-day-bar.

Gassing cheeses, like Asiago, Leerdammer and Emmentaler, were best preserved in a package comprising a support member with an OTR in the range of 80 to 250 cm³/m²-day-bar and a skin-forming flexible film with an OTR in the range of 60 to 300 cm³/m²-day-bar, preferably 100 to 200 cm³ /m²-day-bar.

Typically the materials suitable for both the support member and the flexible skin-forming film have carbon dioxide transmission rates (measured using an analytical technique analogous to ASTM D-3985 at 23°C and 0% RH) greater than 250 cm³/m²-day-bar, preferably greater than 300 cm³/m²-day-bar.

The materials suitable for the support member have OTR values at 23°C and 100% RH (measured using an analytical technique analogous to ASTM D-3985 at 23°C and 0% RH wherein both sides of the specimens to be tested are kept in contact with water for four days before being tested) greater than 100 cm³/m²-day-bar, typically greater than 140 cm³/m² -day-bar.

The OTR values at 23°C and 100% RH of the materials suitable for the flexible skin-forming film are greater than 300 cm³/m²-day-bar, generally greater than 450 cm³/m²-day-bar.

The support member and the flexible skin-forming film are mostly obtained from multi-layer plastic materials. They may include any number of layers from 2 to as many as 20. Preferably they will include from 4 to 15 and more preferably 5 to 10.

The materials to be used for the support member typically require some rigidity and good thermoforming properties whereas the materials to be used for the skin-forming film require stretchability and flexibility.

A key requirement for the skin packaging material in the VSP process is a high degree of formability/stretchability to avoid a common and recurrent problem in such operations, which is the occurrence of wrinkles and other irregularities in the final packaged product.

Typically, plastic materials suitable for the support member of the present invention have a thickness greater than 100, 120, 150, 170, 200 µm.

The thicknesses of materials suitable for the support member are generally less than 1200, 1000, 850, 700 µm.

Plastic materials suitable for the skin-forming film of the present invention have a thickness greater than 35, 50, 60, 70 µm.

The thicknesses of materials suitable for the skin-forming film are less than 200,180, 150, 120 µm.

When the support member and the skin-forming film of the package of the present invention are made of multi-layer thermoplastic materials, they comprise at least one outer layer, optionally one oxygen barrier layer and at least one heat-sealable surface layer.

The oxygen barrier layer, if present, comprises any of the polymers known in the art for their oxygen barrier properties, such as EVOH, PVDC, polyesters, polyamides and blends thereof. Particularly suitable are polyesters, polyamides and blends of polyamides and EVOH in weight ratios from 10:90 to 90:10.

PVDC is any vinylidene chloride copolymer wherein a major amount of the copolymer comprises vinylidene chloride and a minor amount of the copolymer comprises one or more unsaturated monomers copolymerisable therewith, typically vinyl chloride, and alkyl acrylates or methacrylates (e.g. methyl acrylate or methacrylate) and the blends thereof in different proportions. Generally a PVDC barrier layer will contain plasticisers and/or stabilizers as known in the art.

EVOH is the saponified product of ethylene-vinyl ester copolymers, generally of ethylene-vinyl acetate copolymers, wherein the ethylene content is typically comprised between 20 and 60% by mole and the degree of saponification is generally higher than 85% preferably higher than 95%.

Polyamides used as gas barrier layer can be homo- or co-polyamides. This term specifically includes those aliphatic polyamides or copolyamides commonly referred to as e.g. polyamide 6 (homopolymer based on ε-caprolactam), polyamide 69 (homopolycondensate based on hexamethylene diamine and azelaic acid), polyamide 610 (homopolycondensate based on hexamethylene diamine and sebacic acid), polyamide 612 (homopolycondensate based on hexamethylene diamine and dodecandioic acid), polyamide 11 (homopolymer based on 11-aminoundecanoic acid), polyamide 12 (homopolymer based on ω-aminododecanoic acid or on laurolactam), polyamide 6/12 (polyamide copolymer based on ε-caprolactam and laurolactam), polyamide 6/66 (polyamide copolymer based on ε-caprolactam and hexamethylenediamine and adipic acid), polyamide 66/610 (polyamide copolymers based on hexamethylenediamine, adipic acid and sebacic acid), modifications thereof and blends thereof. Said term also includes crystalline or partially crystalline, aromatic or partially aromatic, polyamides, like MXD6/MXDI that is an aromatic copolyamide formed in the reaction between metaxylylenediamine, adipic acid and isophtalic acid.

The term "polyesters" refers to polymers obtained by the polycondensation reaction of dicarboxylic acids with dihydroxy alcohols. Suitable dicarboxylic acids are, for instance, terephthalic acid, isophthalic acid, 2,6-naphthalene dicarboxylic acid and the like. Suitable dihydroxy alcohols are for instance ethylene glycol, diethylene glycol, 1,4-butanediol, 1,4-cyclohexanedimethanol and the like. Examples of useful polyesters include poly(ethylene 2,6-naphtalate), poly(ethylene terephthalate), and copolyesters obtained by reacting one or more dicarboxylic acids with one or more dihydroxy alcohols.

The thickness of the oxygen barrier layer, if present, will be set in order to provide the overall laminate with an OTR at 23°C and 0% RH that is in line with the specific requirements of the type of cheese being packed.

The heat-sealable surface layer comprises materials chosen from the group of ethylene homo-and co-polymers, propylene homo- and co-polymers, ionomers and the like as well as blends of these polymers in any proportions. Suitable blends for the heat-sealable layer also include peelable blends. As used herein, the term "copolymer" refers to a polymer derived from two or more types of monomers, and includes terpolymers. Ethylene homopolymers include high density polyethylene (HDPE) and low density polyethylene (LDPE). Ethylene copolymers include ethylene/alpha-olefin copolymers and ethylene/unsaturated ester copolymers. Ethylene/alpha-olefin copolymers generally include copolymers of ethylene and one or more comonomers selected from C₃ to C₂₀ alpha-olefins, such as 1-butene, 1-pentene, 1-hexene, 1-octene, 4-methyl-1-pentene and the like.

Ethylene/alpha-olefin copolymers generally have a density in the range of from about 0.86 to about 0.94 g/cm³. The term linear low density polyethylene (LLDPE) is generally understood to include that group of ethylene/alpha-olefin copolymers which fall into the density range of about 0.915 to about 0.94 g/cm³ and particularly about 0.915 to about 0.925 g/cm ³. Sometimes linear polyethylene in the density range from about 0.926 to about 0.94 g/cm³ is referred to as linear medium density polyethylene (LMDPE). Lower density ethylene/alpha-olefin copolymers may be referred to as very low density polyethylene (VLDPE) and ultra-low density polyethylene (ULDPE). Ethylene/alpha-olefin copolymers may be obtained by either heterogeneous or homogeneous polymerization processes.

Another useful ethylene copolymer is ethylene/unsaturated ester copolymer, which is the copolymer of ethylene and one or more unsaturated ester monomers. Useful unsaturated esters include vinyl esters of aliphatic carboxylic acids, where the esters have from 4 to 12 carbon atoms, such as vinyl acetate, and alkyl esters of acrylic or methacrylic acid, where the esters have from 4 to 12 carbon atoms.

Useful propylene copolymers include propylene/ethylene copolymers (EPC), which are copolymers of propylene and ethylene having a majority weight percent content of propylene, and propylene/ethylene/butene terpolymers (EPB), which are copolymers of propylene, ethylene and 1-butene.

Preferred materials for the heat-sealable layer are LDPE, ethylene/alpha-olefin copolymers, ionomers, ethylene-vinyl acetate copolymers and blends thereof.

The thickness of the heat-sealable surface layer is typically comprised between 2 and 80 µm, more preferably from about 2 to about 50 µm.

The outer layer comprises materials chosen from the group of ethylene homo-and co-polymers, propylene homo- and co-polymers, ionomers and polyesters.

The thickness of the outer layer is typically comprised between 2 and 400 µm, more preferably from about 2 to about 50 µm.

Other layers can be present in both the support member and the skin-forming film, such as tie or adhesive layers, abuse layers and the like. Said additional layers should serve the purpose of providing the necessary mechanical properties, such as modulus, puncture resistance, abuse resistance, etc. or to improve the bond between the various layers.

A non-limiting example of a suitable multi-layer film for the support member of the package of the present invention is for instance an eight-layer material with an ionomer heat-sealable layer having the following layer composition:

Support # 1:

lo (2 µm) / EVA (9 µm) / Adh (28 µm) / LDPE (144 µm) / Adh (7 µm) /LDPE (11 µm) / Adh (10 µm) / PP (370 µm).

An alternative example can be a ten-layer material with an EVA heat-sealable layer having the following layer composition:

Support # 2:

EVA (2 µm) / EVA (8 µm) / Adh (7µm) / PS (95 µm) / Adh (8 µm) / 50 wt.% PA6/12 + 50 wt.% EVOH (3 µm) / Adh (8 µm) / PS (98 µm) / Adh (12 µm) / PETG (12 µm).

Support # 3:

Same layer sequence as Support # 2 with the following barrier layer composition: 70 wt.% PA6/12 + 30 wt.% EVOH.

Still alternatively a ten-layer material with an EVA heat-sealable layer having the following layer composition:

Support # 4:

EVA (3 µm) / EVA (13 µm) / Adh (11 µm) / PS (140 µm) / Adh (12 µm) / LDPE (12 µm) / Adh (14 µm) / PS (140 µm) / Adh (17 µm) / PETG (18 µm).

Where: lo is an ionomer; EVA is an ethylene-vinyl acetate copolymer; Adh is a tie resin, such as a maleic anhydride-grafted ethylene copolymer; PS is a blend of polystyrene and styrene-butadiene-styrene block copolymer; PP is a propylene homopolymer; PA 6/12 is a polyamide 6/12 and PETG is a copolyester formed in the reaction between terephthalic acid, ethylene glycol and 1,4-cyclohexanedimethanol.

In order to provide the package of the invention with an easy-to-open feature the EVA layer adjacent to the heat-sealable food-contact layer in the materials described above might be replaced with a layer consisting of a blend of resins having a low cohesive strength. Blends with low cohesive strength that can be used are for instance those described in WO99/54398.

The multi-layer materials suitable for both the support member and the skin-forming film are produced using common techniques known in the art such as extrusion, co-extrusion or by heat- or glue-lamination, extrusion coating and the like.

The materials, in particular the materials suitable for the skin-forming film, may be cross-linked. The preferred method of cross-linking is by electron-beam irradiation and is well known in the art. One skilled in the art can readiliy determine the radiation exposure level suitable for a particular application. Generally, however, radiation dosages of up to about 250 kGy, typically between 90 and 220 kGy, with a preferred dosage of between 110 and 200 kGy.

A non-limiting example of a suitable multi-layer film for the skin-forming film of the package of the present invention is for instance a nine-layer material with a LDPE heat-sealable layer having the following layer composition:

Skin-forming film # 1:

LDPE (5 µm) / LDPE (12 µm) / EVA (18 µm) / Adh (3 µm) / PA 6/66 (6 µm) / Adh (4 µm) /EVA (12 µm) / LDPE (28 µm) / HDPE (10 µm).

Or alternatively:

Skin-forming film # 2:

LDPE (6 µm) / LDPE (14 µm) / EVA (19 µm) / Adh (3 µm) / PA 6/66 (10 µm) / Adh (4 µm) /EVA (11 µm) / LDPE (26 µm) / HDPE (10 µm).

Alternatively an eight-layer material with a LLDPE heat-sealable layer ha ving the following layer composition:

Skin-forming film # 3:

LLDPE (13 µm) / EVA (28 µm) / Adh (5 µm) / PA 6/66 (10 µm) / Adh (5 µm) / EVA (28 µm) / Adh (6 µm) / PETG (5 µm).

Where PA6/66 is a polyamide 6/66.

Alternatively an eight-layer material with a LDPE heat-sealable layer having the following layer composition:

Skin-forming film # 4:

LDPE (9 µm) / EVA (5 µm) / EVA (25 µm) / Adh (3 µm) / LDPE (7 µm) / Adh (3 µm) /EVA (36 µm) / HDPE (12 µm).

The oxygen transmission properties of the materials described above are reported in Table 1.

**Table 1**

| Material | OTR 23°C and 0% RH (cm³/m²-day-bar) | OTR 23°C and 100% RH (cm³/m²-day-bar) |
|---|---|---|
| Support # 1 | 135 | 140 |
| Support # 2 | 83 | 200 |
| Support # 3 | 200 | 170 |
| Support # 4 | 220 | 220 |
| Skin-forming film # 1 | 182 | 650 |
| Skin-forming film # 2 | 106 | 456 |
| Skin-forming film # 3 | 97 | 303 |
| Skin-forming film # 4 | 970 | - |

Non-limiting examples of packages according to the present invention are for instance: Support #1 / Emmentaler cheese / Skin-forming film #3; Support #1 / Asiago cheese / Skin-forming film #3; Support #1 / Roquefort cheese / Skin-forming film #4; Support #2 / Leerdammer cheese / Skin-forming film #1.

Packaging tests were performed to evaluate the shelf-life of different gassing cheeses with different support/skin-forming film combinations. Chunks of approximately 200 g of the different cheeses were vacuum skin packaged using different support/skin-forming film combinations and stored at 6-7°C in daylight. Checks were performed 7 or 9 weeks after packaging for gas formation ("ballooning"), visible mould presence inside the packs and odor and taste after unpacking. The results are reported in Table 2.

**Table 2**

| Cheese | Support # | Skin-for ming film # | Weeks | Moulds | Balloning | Odor/Taste change |
|---|---|---|---|---|---|---|
| Asiago | 1 | 3 | 7 | No | No | Slight |
| Asiago | 3 | 1 | 9 | No | No | Slight |
| Asiago | 1 | Comp.* | 7 | No | Yes | Severe |
| Leerdammer | 2 | 1 | 9 | No | No | None |
| Leerdammer | 3 | 1 | 9 | No | No | None |

* Comparative skin-forming film having an OTR value at 23°C and 0% RH and 100% RH of 44 cm³/m²-day-bar and 90 cm³/m²-day-bar, respectively.

In its second aspect the present invention relates to a method of making a vacuum skin package for cheese, said method comprising the steps of:
- providing a support member;
- loading a cheese product over the support member;
- draping a flexible film over the cheese product enclosing said cheese product on the support member, characterized in that the support member has an oxygen transmission rate (measured according to ASTM D-3985) in the range of from 80 to 500 cm³ /m²-day-bar at 23°C and 0% RH and the flexible film has an oxygen transmission rate (measured according to ASTM D-3985) greater than 60 cm³ /m² -day-bar at 23°C and 0% RH.

More in detail, the skin-forming film is fed to the upper section of a heated vacuum chamber comprising an upper and a lower section, and a vacuum is applied thereto from the outside, thereby drawing the skin-forming film into a concave form against the inwardly sloping walls of the upper section of the chamber and against the ports contained in the horizontal wall portion thereof (the top of the dome). Any conventional vacuum pump can be used to apply the vacuum and preferably the skin-forming film is suitably pre-heated prior to the foregoing operation to render it more formable and thus better able to assume a concave shape in the upper section of the vacuum chamber. The product to be packaged is positioned on a support member, that can be flat or shaped, typically tray-shaped, and placed on a platform that is carried in the vacuum chamber, in the lower section thereof, just below the dome. The support member can be shaped off-line or, alternatively, in-line at an initial station on the vacuum packaging machine. Then the vacuum chamber is closed by moving the upper section down onto the lower one and during this whole sequence of operations vacuum is constantly applied to retain the concave shape of the laminate. Once the vacuum chamber is closed, vacuum is applied also in the lower section of the vacuum chamber in order to evacuate the space between the support member and the top skin-forming film. Vacuum in the upper section of the vacuum chamber continues to be applied to retain the concave shape of the skin-forming film until the area between the support and the skin-forming film is evacuated, then it is released and atmospheric pressure is admitted. This will collapse the softened top skin-forming film over the product and the support, as the atmosphere pushing the skin-forming film from the top and the vacuum pulling it from the bottom will cooperatively work to have the skin-forming film substantially conform to the shape of the product to be packaged on the support member. For some types of cheeses, for instance the ones having a sponge-like structure like Asiago, it might be necessary to control the speed of evacuation of the chamber to prevent the collapse of the cheese structure. Optionally, after the evacuation step has been completed, a suitably selected purging gas or gas mixture could be flushed over the product to generate a very low residual gas pressure into the package. In some instances heat-sealing bars or other sealing means can be present in the vacuum chamber to carry out a perimeter heat-seal of the skin-forming film to the support member.

The packaging method of the invention could be performed on currently available VSP machines, like the Multivac® CD6000 or the Multivac® R270.

## Claims

1. A vacuum skin package comprising a) a support member; b) a cheese product loaded onto said support member; and c) a flexible film draped over the cheese product and enclosing said cheese product on the support member, **characterized in that** the support member a) has an oxygen transmission rate (measured according to ASTM D-3985) in the range of from 80 to 500 cm³ /m² -day-bar at 23°C and 0% RH and the flexible film c) has an oxygen transmission rate (measured according to ASTM D-3985) greater than 60 cm³ /m²-day-bar at 23°C and 0% RH.

2. The package according to claim 1 wherein the flexible film is a multi-layer film comprising at least one oxygen barrier layer comprising a polyamide.

3. The package according to claim 1 wherein the support member has an oxygen transmission rate in the range of from 80 to 250 cm³/m²-day-bar at 23°C and 0% RH, the cheese product is a gassing cheese and the flexible film has an oxygen transmission rate in the range of from 60 to 300 cm³/m²-day-bar at 23°C and 0% RH.

4. The package according to claim 1 wherein the flexible film has an oxygen transmission rate greater than 500 cm³/m²-day-bar at 23°C and 0% RH and the cheese product is a moulded cheese.

5. The package according to claim 1 wherein the support member has an oxygen transmission rate in the range of from 80 to 500 cm³/m²-day-bar at 23°C and 0% RH, the cheese product is a moulded cheese and the flexible film has an oxygen transmission rate in the range of from 500 to 1000 cm³/m²-day-bar at 23°C and 0% RH.

6. A method of making a vacuum skin package for cheese comprising the steps of: providing a support member; loading a cheese product over the support member; draping a flexible film over the cheese product enclosing said cheese product on the support member, **characterized in that** the support member has an oxygen transmission rate (measured according to ASTM D-3985) in the range of from 80 to 500 cm³ /m²-day-bar at 23°C and 0% RH and the flexible film has an oxygen transmission rate (measured according to ASTM D-3985) greater than 60 cm³ /m²-day-bar at 23°C and 0% RH.
